# NEW EUROPEAN PATENT SPECIFICATION

(11) **EP 0 232 770 B2**
(45) Date of publication and mention of the opposition decision: **18.06.1997**
(45) Mention of the grant of the patent: 07.04.1993
(21) Application number: 87100941.1
(22) Date of filing: 23.01.1987
(51) Int. Cl.: G03C 7/26, G03C 7/30, G03C 7/38

(54) **Method of the formation of color images**
Verfahren zur Herstellung von Farbbildern
Méthode pour former des images couleur

(30) Priority: 24.01.1986 JP 14546/86
(43) Date of publication of application: 19.08.1987
(73) Proprietor: FUJI PHOTO FILM CO., LTD., Kanagawa-ken, 250-01 (JP)
(72) Inventor: Takahashi, Osamu c/o Fuji Photo Film Co., Ltd., Kanagawa-ken (JP); Naruse, Hideaki c/o Fuji Photo Film Co., Ltd., Kanagawa-ken (JP); Sakai, Nobuo c/o Fuji Photo Film Co., Ltd., Kanagawa-ken (JP)
(74) Representative: Grünecker, Kinkeldey, Stockmair & Schwanhäusser Anwaltssozietät

(56) References cited:
- EP-A- 0 080 896
- EP-A- 0 080 905
- EP-A- 0 081 768
- EP-A- 0 107 488
- EP-A- 0 112 545
- EP-A- 0 119 741
- EP-A- 0 119 860
- EP-A- 0 162 328
- EP-A- 0 164 961
- DD-A- 215 642
- DD-A- 217 330
- DD-A- 221 854
- GB-A- 2 140 572
- PATENT ABSTRACTS OF JAPAN, vol. 9, no. 308 (P-410)[2031], 4th December 1985
- PATENT ABSTRACTS OF JAPAN, vol. 5, no. 56 (P-57)[728], 17th April 1981
- PATENT ABSTRACTS OF JAPAN, vol. 3, no. 18 (E-91), 16th February 1979, page 71 E91
- CHEMICAL ABSTRACTS, vol. 101, no. 20, November 1984, page 625, no. 181073y, Columbus, Ohio, US

## Description

The present invention relates to a method for the formation of color images on silver halide color photographic materials and, in particular, to using improved color couplers without the use of benzyl alcohol for the reduction of processing time.

A silver halide color photographic material has a multilayer light-sensitive film, as coated on a support, comprising three kinds of silver halide emulsion layers selectively sensitized so that the layers may have a light sensitivity to blue light, green light and red light, individually. For instance, a so-called color photographic paper (hereinafter referred to as "color paper") generally has a red-sensitive emulsion layer, a green-sensitive emulsion layer and a blue-sensitive emulsion layer as coated on a support to be exposed to light and, in addition, for example color stain preventive or ultraviolet absorptive intermediate layers and protective layers, are provided between the light-sensitive layers.

For the formation of color photographic images, photographic couplers for the three colors of yellow, magenta and cyan are incorporated into the light-sensitive layers and the photographic materials are, after having been exposed to light, subjected to color development with a so-called color developing agent. The coupling reaction between the oxidized product of an aromatic primary amine and the coupler results in the formation of colored dyes. Coupling speed in the reaction as high as possible and the couplers having higher colorability so as to obtain a higher color density within the limited developing time are desired. Moreover, the colored dyes are required to be sharp cyan, magenta, and yellow dyes, individually, with less side absorption and to form color photographic images of good color reproduceability.

On the other hand, the color photographic images as formed are required to have good preservation stability under various conditions. In order to satisfy this requirement, it is important that the discoloration or color change speed of the colored dyes of different hues is slow and that the discoloration speed is as even as possible throughout the whole range of the color image density with less variation of the color balance of the remaining color image.

In order to solve these problems, so-called oil-soluble couplers have heretofore been proposed, which are dissolved in a high boiling or low boiling organic solvent, and the resulting coupler solution is emulsified, dispersed, and incorporated into an emulsion layer. The use of such couplers, however, is accompanied by difficult problems such as the color developing agent hardly penetrating into the coupler dispersion-containing oil drops, the agent having a poor oleophilic property, and low color density. Under these circumstances, various kinds of developing agent-penetratives have been investigated. In particular, the addition of benzyl alcohol to color developers for the acceleration of the color development has heretofore been widely utilized for the processing of photographic color photographic materials, in particular, color papers, as the coloration-accelerating effect by the addition of benzyl alcohol is remarkable.

However, the use of benzyl alcohol requires diethylene glycol, triethylene glycol or alkanolamines as a solvent, since benzyl alcohol has poor water solubility. Benzyl alcohol and these solvents have high BOD and COD values, which are environmental pollution load values, and, therefore, the elimination of benzyl alcohol is preferable in view of the need to reduce the environmental pollution load.

Moreover, even when such solvents are used, the dissolution of benzyl alcohol in the solvents requires much time and, therefore, the use of benzyl alcohol is not preferred, because it is desirable to reduce the time required for preparation of photographic processing solutions.

Further, in the case where benzyl alcohol is carried over into the bleaching bath or bleach-fixing bath, which is a post-bath after the developing bath, this will result in the formation of a leuco dye of a cyan dye, causing a decrease in color density. In addition, the use of benzyl alcohol will retard the rate at which developer components are washed out, which often adversely influences the image preservation stability of photographic materials after processing. Accordingly, benzyl alcohol is preferably not used in view of the above-mentioned reasons.

Color development is, in general, completed within 3 to 4 minutes by conventional means and, recently, reduction of processing time is being required along with the reduction of the time limit for the delivery of commercial color prints and with the reduction of the development laboratory work load.

In spite of this situation, the elimination of benzyl alcohol, which is a coloration accelerator, and reduction of the developing time have not been possible without causing an inevitably noticeable deterioration of color density.

In order to solve these problems, various kinds of color development accelerators (for example, compounds as described in U.S. Patents 2,950,970, 2,515,147, 2,496,903, 2,304,925, 4,038,075 and 4,119,462, British Patents 1,430,998 and 1,455,413, Japanese Patent Application (OPI) Nos. 15831/78, 62450/80, 62451/80, 62452/80 and 62453/80 (the term "OPI" as used herein refers to a "published unexamined Japanese patent application"), and Japanese Patent Publication Nos. 12422/76 and 49728/80) have heretofore been tried to be co-used together with color developers, but sufficient color density could not be obtained as yet.

The incorporation of 3-pyrazolidones into photographic materials (for example, as described in Japanese Patent Application (OPI) Nos. 26338/85, 158444/85 and 158446/85) still is defective in that the sensitivity of the photographic materials is lowered and fog occurs during the formation of the photographic materials.

The incorporation of color developing agents into photographic materials (for example, as described in U.S. Patents 3.719,492, 3.342,559 and 3,342,597 and Japanese Patent Application (OPI) Nos. 6235/81, 16133/81, 97531/82 and 83565/82) also is defective in that the speed of the color development is lowered and fog occurs, and this is undesirable.

In order to overcome these problems, the use of silver chloride emulsions (for example, as described in Japanese Patent Application (OPI) Nos. 95345/83, 232342/84 and 19140/85) has been provided.

Furthermore, in the conventional method for the formation of color images wherein a reflective silver halide photographic material is processed by using a color developer which does not contain benzyl alcohol or contains little benzyl alcohol, high boiling organic solvents used as coupler solvents are as follows; dibutyl phthalate (for example, as described in Japanese Patent Application (OPI) Nos. 200037/82, 50536/83, 48755/84, 177553/84 and 162256/85, and Japanese Patent Publication No. 29461/74), dioctyl phthalate (for example, as described in Japanese Patent Application (OPI) Nos. 26338/85, 26339/85, 158446/85 and 172042/85), tricresyl phosphate (for example, as described in Japanese Patent Application (OPI) Nos. 200037/82 and 50536/83, and Japanese Patent Publication No. 29461/74), dioctylbutyl phosphate (for example, as described in Japanese Patent Application (OPI) No. 50536/83), and trioctyl phosphate (for example, as described in Japanese Patent Application (OPI) Nos. 174836/84, 177553/84 and 162256/85).

However, a method for the formation of still more sufficient color images in a still shorter period of time by using color developers which do not substantially contain benzyl alcohol has not heretofore been found as yet.

Accordingly, it is the object of the present invention to provide a method for the formation of color images in a short period of time by processing color photographic materials containing at least one oil-soluble coupler with color developers which do not substantially contain benzyl alcohol, and the color images formed by this method should have good color reproducibility and high color image preservation stability.

The object of the present invention can be achieved by the provision of a method for the formation of color images comprising image-wise exposing a silver halide color photographic material having at least one silver halide emulsion layer on a reflective support, said emulsion layer containing a dispersion of oleophilic fine grains having a mean grain size of 0.05 to 0.25 µm which dispersion contains a pyrazolo[5,1-c][1,2,4]triazole or pyrazolo [1,5-b][1,2,4]triazole coupler capable of forming a magenta dye after having been coupled with an oxidation product of an aromatic primary amine developing agent, and at least one high boiling organic solvent having a dielectric constant of 5.0 or more (25°C, 10 kHz) and having the following formula (I) wherein W₁, W₂ and W₃ each represents a substituted or unsubstituted alkyl, cycloalkyl, alkenyl, aryl or heterocyclic group; and then subjecting the imagewise exposed photographic material to development with a color developer which contains an aromatic primary amine developing agent and 0.5 ml/l or less of benzyl alcohol, for a period of time within 2 min and 30 s or less.

In the present invention the concentration of benzyl alcohol in the color developer is 0.5 ml/l or less and, in particular, it is preferred that no benzyl alcohol is contained in the color developer.

The mean grain size is measured by the dynamic light scattering photometric method.

Preferred substances represented by the above-mentioned formula (I) are those, in which the total of the carbon atoms in W₁, W₂ and W₃ is about 8 or more.

The dielectric constant can easily be obtained by measuring by means of the transformer bridge method. When these W₁, W₂ and W₃ have substituents, the substituents may contain one or more linking groups selected from -COO-, -CON〈, -R⁸-N〈, and -O-, where R⁸ represents a divalent to hexavalent group derived from a phenyl group by removal of hydrogen atom(s) therefrom.

In the formula (I) the alkyl group as represented by W₁, W₂ or W₃ may be either linear or branched, and include, for example, a methyl group, an ethyl group, a propyl group, a butyl group, a pentyl group, a hexyl group, a heptyl group, an octyl group, a nonyl group, a decyl group, an undecyl group, a dodecyl group, a tridecyl group, a tetradecyl group, a pentadecyl group, a hexadecyl group, a heptadecyl group, an octadecyl group, a nonadecyl group or an eicosyl group.

Substituents for these alkyl groups are, for example, halogen atoms, cycloalkyl groups, aryl groups and ester groups, and examples of the substituted alkyl groups include:

Halogen-substituted (such as F-, Cℓ- or Br-substituted) groups such as -C₂HF₄, -C₅H₃F₈, -C₉H₃F₁₆, -C₂H₄Cℓ, -C₃H₆Cℓ, -C₃H₅Cℓ₂, -C₃H₅CℓBr, or -C₃H₅Br₂;

Cycloalkyl-substituted groups such as

Aryl-substituted groups such as

Dibasic acid ester-forming groups such as -CH₂CH₂COOC₁₂H₂₅, or

Lactate-forming groups such as

Citrate-forming groups such as

Malate-forming groups such as -CH₂CH(OH)-COOC₆H₁₃;
Tartrate-forming groups such as -CH(OH)CH(OH)COOC₈H₁₇, or and

The group of

The cycloalkyl group represented by W₁, W₂ or W₃ is, for example, and the substituted cyclohexyl group represented by W₁, W₂ or W₃ is, for example,

The aryl group represented by W₁, W₂ or W₃ includes, for example, aromatic, substituted or unsubstituted, fused or nonfused, 6-membered rings such as and the substituted aryl group represented by the same is, for example, or

Alkenyl groups include for example -C₄H₇, -c₅H₉, -C₆H₁₁, -C₇H₁₃, -C₈H₁₅, -C₁₀H₁₉, -C₁₂H₂₃ and -C₁₈H₃₅; and substituted alkenyl groups include, for example, those substituted by a halogen atom (e.g., F, Cℓ, Br), -OC₈H₁₇, -OC₁₂H₂₅, -OCOC₈H₁₇, and -C₈H₁₅, -C₁₂H₂₃, or include for example

The unsubstituted or substituted heterocyclic group represented by W₁, W₂ or W₃, includes, for example,

Preferably, the high boiling organic solvents have a viscosity of 20 mPa.s or more at 25°C. It is surprising that compounds satisfying these conditions can improve the colorability of coloring dyes without deteriorating the absorbance and other characteristics of the dyes. Though the reason for these results is not clear, it is assumed that the high boiling organic solvents having a high dielectric constant can accept a large amount of the color developing agents and those having a viscosity of 20 mPa.s or more at 25°C can reduce some adverse effects of the couplers and the silver halides in the oil droplets.

In the present invention, the amount of the high boiling organic solvent represented by the formula (I), may be any desired amount, depending upon the kinds and the amounts of the couplers used. The ratio by weight of the high boiling solvent/coupler falls, preferably, in the range of 0.05 to 20. The high boiling organic solvents of the formula (I) can be used singly or in the form of a mixture of two or more of them.

Specific examples of the high boiling organic solvents are given below.

### (S-1)

O = P⁅O-(n-C₄H₉)]₃

### (S-2)

### (S-3)

O = P⁅O-(n-C₆H₁₃)]₃

### (S-4)

### (S-5)

### (S-8)

### (S-16)

### (S-17)

### (S-18)

### (S-19)

### (S-20)

### (S-21)

### (S-22)

The oleophilic fine grains to be used in the present invention can be obtained, in general, by a method where a solution of the compound dissolved in a substantially water-insoluble high boiling organic solvent and a hydrophilic colloid solution are blended and dispersed. This method is described, for example, in U.S. Patents 2,322,027, 2,533,514 and 2,801,171. If necessary, a low boiling solvent or a water-miscible organic solvent can be used, and these solvents are removed by drying evaporation or water-washing. In the case of this method, a surfactant is preferably co-used. In general, the reduction of the grain size of the above-mentioned oleophilic fine grains can be attained by the ingenuity in the apparatus or the operation, including the selection of the kinds of surfactants, the increment of the amount of the surfactant to be used, the increment of the viscosity of the hydrophilic colloid solution, the reduction of the viscosity of the organic layer in which the above-mentioned compound has been dissolved by the co-use of the low boiling solvent, the elevation of the rotation of the stirring blades in the emulsifier to reinforce the cutting force, and increasing emulsifying time. Other methods for the preparation of the oleophilic fine grain dispersion, for example, as described in U.S. Patent 3,619,195, West German Patent (OAS) No. 1,957,467 and Japanese Patent Application (OPI) No. 59943/76, can also be utilized. Preferred surfactants are described, for example, in Japanese Patent Publication No. 4923/84 and U.S. Patent 3,676,141.

Particularly preferred surfactants are the following compounds having an aliphatic group and a sulfonic acid group.
(i) and
(ii)

These may be used alone or in combination thereof.

The grain size of the oleophilic fine grains of the present invention is preferably 0.05 µm to 0.20 µm.

The oleophilic fine grains may contain, in addition to the coupler, a discoloration inhibitor, an ultraviolet absorbent, a DIR coupler and the like oleophilic photographic elements.

The "reflective support" to be used in the present invention is one having an improved reflectivity, which has a function to improve the sharpness of the color image as formed in the silver halide emulsion layer. Examples of such reflective supports include those formed by coating a hydrophobic resin which contains a dispersion of a light-reflective substance such as titanium oxide, zinc oxide, calcium carbonate or calcium sulfate, on a support, or those made of a hydrophobic resin containing a dispersion of such a light-reflective substance. For instance, baryta paper, polyethylene-coated paper, polypropylene type synthetic paper, as well as transparent supports on which a reflective layer has been provided or in which a reflective substance has been incorporated such as a lass plate, polyethylene terephthalate, cellulose triacetate, cellulose nitrate and the like polyester films, and polyamide films polycarbonate films and polystyrene films can be used. These supports can properly be selected in accordance with the use and the object of the photographic materials.

Next, the photographic processing step (image-forming step) in the present invention will be described hereunder.

The color development step in the present invention progresses rapidly: The processing time is 2 min and 30 s or less. The preferred processing time is 1 to 2 min . "Processing time" means the time from the first contact of the photographic material to be processed with color developer to contact of the material with the next bath, including the time for the transference of the material between the baths.

The color developer to be used in the present invention is preferably an alkaline aqueous solution mainly comprising an aromatic primary amine type color developing agent. Paraphenylenediamine type compounds are preferably used as the color developing agent and typical examples thereof are 3-methyl-4-amino-N.N-diethylaniline, 3-methyl-4-amino-N-ethyl-N-β-hydroxyethylaniline, 3-methyl-4-amino-N-ethyl-N-β-methanesulfonamidoethylaniline, 3-methyl-4-amino-N-ethyl-N-β-methoxyethylaniline and sulfates, hydrochlorides, phosphates, p-toluenesulfonates, tetraphenyl borates and p-(t-octyl)benzenesulfonates thereof. Among these, 3-methyl-4-amino-N-ethyl-N-β-hydroxyethylaniline, and 3-methyl-4-amino-N-ethyl-N-β-methanesulfonamidoethylaniline, are preferred, and in particular, 3-methyl-4-amino-N-ethyl-N-β-methanesuIfonamidoethylaniline, is especially preferred.

Aminophenyl type derivatives include, for example, o-aminophenol, p-aminophenol, 4-amino-2-methylphenol, 2-amino-3-methylphenol and 2-hydroxy-3-amino-1,4-dimethylbenzene.

In addition, compounds as described in L.F.A. Mason, Photographic Processing Chemistry, pp. 226 to 229 (Focal Press), U.S. Patents 2,193,015 and 2,592,364, and Japanese Patent Application (OPI) No. 64933/73 can also be used. If necessary, two or more color developing agents can be used in combination.

The processing temperature of the color developer of the present invention is preferably 30 to 50"fl, more preferably 33 to 45°C.

As the development accelerator, any compounds can be used so far as these do not substantially contain benzyl alcohol. For instance, various kinds of pyridinium compounds and other cationic compounds, cationic dyes such as phenosafranine, neutral salts such as thallium nitrate and potassium nitrate, as described in U.S. Patent 2,648,604, Japanese Patent Publication No. 9503/69 and U.S. Patent 3,171,247; nonionic compounds such as polyethylene glycol and derivatives thereof and polythioethers, as described in Japanese Patent Publication No. 9304/69, U.S. Patents 2,533,990, 2,531,832, 2,950,970 and 2,577,127; thioether type compounds as described in U.S. Patent 3,201,242; and compounds as described in Japanese Patent Application (OPI) Nos. 156934/83 and 220344/85 can be mentioned.

In the short time development of the present invention, not only the means for the acceleration of the development but also the technique for the prevention of the development fog is an important subject.

A fog inhibitor may be used in the color developer of the present invention. Alkali metal halides such as potassium bromide, sodium bromide and potassium iodide and organic fog inhibitors are preferably used as the fog inhibitor in the present invention. Examples of usable organic fog inhibitors are nitrogen-containing heterocyclic compounds such as benzotriazole, 6-nitrobenzimidazole, 5-nitrosoindazole, 5-methylbenzotriazole, 5-nitrobenzotriazole, 5-chlorobenzotriazole, 2-thiazolylbenzimidazole, 2-thiazolylmethylbenzimidazole, hydroxyazaindolizine; mercapto-substituted heterocyclic compounds such as 1-phenyl-5-mercaptotetrazole, 2-mercaptobenzimidazole, 2-mercaptobenzothiazole; and, additionally, mercapto-substituted aromatic compounds such as thiosalicylic acid. In particular, the halides are especially preferred. The fog inhibitor can be dissolved out from the color photographic material, while the material is being processed, to be deposited in the color developer solution.

The color developer of the present invention may further contain pH buffers such as alkali metal carbonates, borates or phosphates; preservatives such as hydroxylamines, triethanolamines, compounds as described in DE-A- 2,622,950, sulfites or bisulfites; organic solvents such as diethylene glycol; dye-forming couplers; competing couplers; nucleating agents such as sodium borohydride; auxiliary developing agents such as 1-phenyl-3-pyrazolidone; tackifiers; and chelating agents such as aminopolycarboxylic acids, e.g., ethylenediaminetetraacetic acid, nitrilotriacetic acid, cyclohexanediaminetetraacetic acid, iminodiacetic acid, N-hydroxymethylethylenediaminetriacetic acid, diethylenetriaminepentaacetic acid, triethylenetetraminehexaacetic acid and compounds as described in Japanese Patent Application (OPI) No. 195845/83, 1-hydroxyethylidene-1,1'-diphosphonic acid, organic phosphonic acids as described in Research Disclosure, RD No. 18170 (May, 1979), aminophosphonic acids, e.g., aminotris(methylenephosphonic acid) and ethylenediamine-N,N,N',N'-tetramethylenephosphonic acid and phosphonocarboxylic acids as described in Japanese Patent Application (OPI) Nos. 102726/77, 42730/78, 121127/79, 4024/80, 4025/80, 126241/80, 65955/80 and 65956/80 and Research Disclosure, RD No. 18170 (May, 1979).

If necessary, the color development line may comprise two or more color developer baths and a color developer replenisher can be replenished in the first prebath or in the last postbath whereby the development time can be reduced and the amount of the replenisher may be reduced.

The silver halide color photographic materials are, after having been color-developed, generally bleached. The bleaching can be carried out simultaneously with fixation (bleach-fixing) or, alternatively, separately therefrom. As the bleaching agent there can be used, for example, compounds of polyvalent metals such as iron (III), cobalt (III), chromium (VI) or copper (II), peracids, quinones and nitroso compounds. For instance, ferricyanides, bichromates, organic complexes with iron (III) or cobalt (III) such as complexes of ethylenediaminetetraacetic acid, diethylenetriaminepentaacetic acid, nitrilotriacetic acid, 1,3-diamino-2-propanoltetraacetic acid or the like aminopolycarboxylic acids or with citric acid, tartaric acid, malic acid or the like organic acids, persulfates; manganates; and nitrosophenol can be used. In particular, potassium ferricyanide, sodium ethylenediaminetetraacetate/iron (III), ammonium ethylenediaminetetraacetate/iron (III), ammonium triethylenetetraminepentaacetate/iron (III) and persulfates are especially preferred. Ethylenediaminetetraacetate/iron (III) complexes are usable both in an independent bleaching solution and in a combined bleach-fixing solution.

The bleaching solution and the bleach-fixing solution may contain, if necessary, various kinds of accelerators. For instance, a bromide ion, an iodide ion, as well as thiourea type compounds as described in U.S. Patent 3,706,561, Japanese Patent Publication Nos. 8506/70 and 26586/74, Japanese Patent Application (OPI) Nos. 32735/78, 36233/78 and 37016/78; thiol type compounds as described in Japanese Patent Application (OPI) Nos. 124424/78, 95631/78, 57831/78, 32736/78, 65732/78 and 52534/79 and U.S. Patent 3,893,858; heterocyclic compounds as described in Japanese Patent Application (OPI) Nos. 59644/74, 140129/75, 28426/78, 141623/78, 104232/78 and 35727/79; thioether type compounds as described in Japanese Patent Application (OPI) Nos. 20832/77, 25064/80 and 26506/80; quaternary amines as described in Japanese Patent Application (OPI) No. 84440/73; and thiocarbamoyl type compounds as described in Japanese Patent Application (OPI) No. 42349/74 can be used.

As the fixing agents can be mentioned thiosulfates, thiocyanates, thioether type compounds, thioureas, and a large amount of iodides. In particular, thiosulfates are generally used. As the preservative for the bleach-fixing solution or the fixing solution, sulfites or bisulfites or carbonyl-bisulfuric acid adducts are preferred.

After the bleach-fixing or the fixing, the photographic materials are generally rinsed. In the rinsing step, various kinds of known compounds can be used for the purpose of the prevention of precipitation or of the economization of water. For instance, hard water softeners such as inorganic phosphoric acids, aminopolycarboxylic acids or organic phosphoric acids; bactericides or fungicides for the prevention of growth of various bacteria algae or fungi; hardeners such as magnesium salts or aluminum salts and surfactants for the prevention of drying load or unevenness can be added in need thereof. As the case may be, compounds as described in L.E. West, Photographic Science and Engineering. Vol. 9, No. 6 (1965) can be added. In particular, the addition of the chelating agent or fungicide is effective. A multistage (e.g., two-stage to five-stage) countercurrent flow system can be applied to the rinsing step for the purpose of the economization of water.

After the rinsing step or in place of the rinsing step, the photographic material may be subjected to multistage countercurrent stabilization system as described in Japanese Patent Application (OPI) No. 8543/82. This step requires a countercurrent system bath line comprising two to nine baths. Various kind of compounds are added to the stabilization baths for the stabilization of images. For instance, a pH-regulating buffers (such as borates, metaborates, borax, phosphates, carbonates. potassium hydroxide, sodium hydroxide, aqueous ammonia, monocarboxylic acids, dicarboxylic acids and polycarboxylic acids) and formalin can be added. In addition, hard water softeners (such as inorganic phosphoric acids, aminopolycarboxylic acids, organic phosphoric acids, aminopolyphosphonic acids and phosphonocarboxylic acids), bactericides (such as Proxel, isothiazolone, 4-thiazolylbenzimidazole and halogenated phenol-benzotriazoles), surfactants, fluorescent whiteners, and hardeners, can further be added in need thereof.

Various kinds of ammonium salts such as ammonium chloride, ammonium nitrate, ammonium sulfate, ammonium phosphate. ammonium sulfite, or ammonium thiosulfate can be added as a film pH-regulator for regulating the pH value of the film after processing.

Pyrazoloazole type couplers which are used in the present invention include pyrazolo[5,1-c][1,2,4]triazoles as described in U.S. Patent 3,725,067 and pyrazolo[1,5-b][1,2,4]-triazoles as described in European Patent 119,860. Other color couplers may be additionally used.

The color coupler to be additionally incorporated in the photographic materials preferably has a ballast group or is polymerized to be nondiffusible. 2-Equivalent color couplers where the coupling active positions are substituted by coupling off groups are preferred to 4-equivalent color couplers having hydrogen atoms in the coupling active positions, since the amount of the silver to be coated can be reduced. Further, couplers to form colored dyes with pertinent diffusibility, non-coloring couplers. DIR couplers to release a development inhibitor in the coupling reaction, and couplers to release a development accelerator in the coupling reaction can also be used.

Typical examples of yellow couplers which can be additionally used in the present invention are oil-protected acylacetamide type couplers. Specific examples thereof are described in U.S. Patents 2,407,210, 2,875,057 and 3,265,506. In the present invention, 2-equivalent yellow couplers are preferably used, and typical examples thereof are oxygen atom-coupling off type yellow couplers as described in U.S. Patents 3,408,194, 3,447,928, 3,933,501 and 4,022,620 and nitrogen atom-coupling off type yellow couplers as described in Japanese Patent Publication No. 10739/83, U.S. Patents 4,401,752 and 4,326,024, Research Disclosure, RD No. 18053 (April, 1979), British Patent 1,425,020 and DE-A- 2,219,917, 2,261,361, 2,329,587 and 2,433,812, α-Pivaloylacetanilide type couplers are excellent in fastness, especially to light, of the colored dyes. On the other hand, α-benzoylacetanilide type couplers are excellent in producing high color density.

Magenta couplers which can be additionally used in the present invention include oil-protected indazolone type or cyanoacetyl type couplers, preferably 5-pyrazolone type couplers and pyrazoloazole type couplers such as pyrazolotriazoles. Among the 5-pyrazolone type couplers, those whose 3-position is substituted by an arylamino group or an acylamino group are preferred in view of the hue and the color density of the colored dyes. Typical examples of these couplers are described in U.S. Patents 2,311,082, 2,343,703, 2,600,788, 2,908,573, 3,062,653, 3,152,896 and 3,936,015. Regarding the coupling off groups of the 2-equivalent 5-pyrazolone type couplers, nitrogen atom-coupling off groups as described in U.S. Patent 4,310,619 and arylthio groups as described in U.S. Patent 4,351,897 are especially preferred. In addition, ballast group-containing 5-pyrazolone type couplers as described in European Patent 73.636 are preferred, as forming color images of high color density.

Pyrazolotetrazoles as described in Research Disclosure, RD No. 24220 (June 1984) and pyrazolopyrazoles as described in Research Disclosure, RD No. 24230 (June 1984) are preferred. In particular, imidazo[1,2-b]pyrazoles as described in European Patent 119,741 are preferred because the yellow side absorption of the dyes formed is small and the light fastness thereof is high.

Cyan couplers which can be additionally used in the present invention are oil-protected naphthol type and phenol type couplers. Typical examples thereof are naphthol type couplers as described in U.S. Patent 2,474,293, preferably oxygen atom-coupling off type 2-equivalent naphthol type couplers as described in U.S. Patents 4,052,212, 4,146,396, 4,228,233 and 4,296,200. Specific examples of phenol type couplers are described in U.S. Patents 2,369,929, 2,801,171, 2,772,162 and 2,895,826. Cyan couplers which are fast to moisture and temperature are preferably used in the present invention, and typical examples thereof are phenol type cyan couplers where the phenol nucleus has an ethyl or a higher alkyl group in the m-position as described in U.S. Patent 3,772,002: 2,5-diacylamino-substituted phenol type couplers as described in U.S. Patents 2,772,162, 3,758,308, 4,125,396, 4,334,011 and 4,327,173, DE-A- 3,329,729 and Japanese Patent Application (OPl) No. 166956/84; and phenol type couplers having a 2-ureido group and a 5-acylamino group as described in U.S. Patents 3,446,622, 4,333,999, 4,451,559 and 4,427,767.

The graininess can be improved by the incorporation of a coupler capable of forming a colored dye with appropriate diffusibility. Such dye-diffusible couplers are magenta couplers as described in U.S. Patent 4,366,237 and British Patent 2,125,570 and yellow, magenta or cyan couplers as described in European Patent 96,570 and DE-A- 3,234,533.

The dye-forming couplers and the above-mentioned special couplers may be in the form of a dimer or more polymer. Typical examples of the polymerized dye-forming couplers are described in U.S. Patents 3,451,820 and 4,080,211. Specific examples of polymerized magenta couplers are described in British Patent 2,102,173 and U.S. Patent 4,367,282.

Regarding the incorporation of the couplers in the photographic materials of the present invention, two or more kinds of the couplers can be incorporated in the same layer of the light-sensitive layer, or the same compound can be incorporated in two or more different layers, so that the photographic material can have the necessary characteristics.

The standard amount of the color coupler to be used is within 0.001 to 1 mol per mol of the light-sensitive silver halide, and preferably the amount of the yellow coupler is 0.01 to 0.5 mol, that of the magenta coupler is 0.003 to 0.3 mol and that of the cyan coupler is 0.002 to 0.3 mol, each per mol of the silver halide.

The photographic light-sensitive material used in the present invention can for example contain hydroquinone derivatives. aminophenol derivatives. amines, gallic acid derivatives, catechol derivatives, ascorbic acid derivatives, non-coloring couplers and sulfonamidophenol derivatives as a color fog inhibitor or color stain preventing agent.

The photographic light-sensitive materials used in the present invention can contain a known discoloration inhibitor. Typical examples of usable organic discoloration inhibitors are hindered phenols such as hydroquinones. 6-hydroxychromans. 5-hydroxycoumarans, spirochromans. p-alkoxyphenols and bisphenols, and gallic acid derivatives, methylenedioxybenzenes. aminophenols. hindered amines. as well as ether and ester derivatives thereof where the phenolic hydroxyl group is silylated or alkylated. In addition, metal complexes such as (bissalicylaldoximato)nickel complexes and (bis-N,N-dialkyldithiocarbamato)nickel complexes can also be used.

Compounds having both partial structures of hindered amine and hindered phenol in one molecule as described in U.S. Patent 4,268,593 are effective for the prevention of the deterioration of the yellow-colored images under heat, moisture and light. Spiroindanes as described in Japanese Patent Application (OPI) No. 159644/81 and hydroquinone-diether- or hydroquinone-monoether-substituted chromans are effective for the prevention or the deterioration of the magenta-colored images, especially under light.

Benzotriazole type ultraviolet absorbents are preferably used for improving preservation stability, especially light fastness, of the cyan-colored images. The ultraviolet absorbent can be co-emulsified with the cyan coupler.

The amount of the ultraviolet absorbent to be coated is enough to be satisfactory for imparting the light stability to the cyan-colored images. If, however, the amount is too large, the non-exposed part (white background part) of the color photographic material will be yellowed and, therefore, the amount is, in general. preferably to fall within the range of 1 x 10⁻⁴ mol/m² to 2 X 10⁻³ mol/m², especially 5 x 10⁻⁴ mol/m² to 1,5 x 10⁻³ mol/m².

In the construction of the light-sensitive layer of general color papers, the ultraviolet absorbent is incorporated into either one, preferably both, of the layers as adjacent to the both sides of the cyan coupler-containing red-sensitive emulsion layer. When the ultraviolet absorbent is added to the intermediate layer between the green-sensitive layer and the red-sensitive layer, this may be co-emulsified with the color stain preventing agent. When the ultraviolet absorbent is added to the protective layer, another protective layer can be provided as an outermost layer. The protective layer can for example contain a matting agent having any desired grain size.

The photographic light-sensitive materials used in the present invention can contain the ultraviolet absorbent in the hydrophilic colloid layer.

The photographic light-sensitive materials used in the present invention can contain a water-soluble dye in the hydrophilic colloid layer as a filter dye or for irradiation prevention or halation prevention or for other various purposes.

The photographic light-sensitive materials used in the present invention can contain whitening agents such as stilbene type, triazine type, oxazole type and coumarin type compounds in the photographic emulsion layers or in other hydrophilic colloid layers. The whitening agents to be used may be water-soluble or, as the case may be, water-insoluble whitening agents can be used in the form of a dispersion thereof.

As mentioned above, the present invention can be adopted to multilayer and multicolor photographic materials having at least two layers of different spectral sensitivities on a support. Multilayer natural color photographic materials have, in general, at least one red-sensitive emulsion layer, at least one green-sensitive emulsion layer and at least one blue-sensitive emulsion layer on a support. The order of these layers to be provided on the support can be selected freely in need thereof. Each of the emulsion layers may comprise two or more layers having different degrees of sensitivity or a light-insensitive layer may be provided between two or more layers, having the same color sensitivity.

The photographic light-sensitive materials used in the present invention preferably have auxiliary layers such as a protective layer, intermediate layer, filter layer, antihalation layer and backing layer, in addition to the silver halide emulsion layers, when needed.

Gelatin is advantageously used as the binder or protective colloid to be incorporated into the emulsion layer or intermediate layer of the photographic light-sensitive materials of the present invention, and other hydrophilic colloids can, of course, be used.

For instance, proteins such as gelatin derivatives, graft polymers of gelatin, and other high molecular weight substances, proteins such as albumin and casein; cellulose derivatives such as hydroxyethyl cellulose, carboxymethyl cellulose and cellulose sulfates; saccharide derivatives such as sodium alginate and starch derivatives; mono- co copolymers various synthetic hydrophilic high molecular weight substances such as polyvinyl alcohol, partially acetalized polyvinyl alcohol, poly-N-vinylpyrrolidone, polyacrylic acid, polymethacrylic acid, polyacrylamide, polyvinyl imidazole and polyvinyl pyrazole, can be used.

Gelatins which can be used in the present invention include lime-treated gelatin, acid-treated gelatin and enzyme-treated gelatin as described in Bull. Scc, Sci. Phot. Japan, No. 16, page 30 (1966); and in addition, hydrolyzed or enzyme-decomposed products of gelatins can also be used.

The photographic light-sensitive materials used in the present invention can further contain, in addition to the above-mentioned additives, various kinds of stabilizers, stain inhibitors, developing agents or precursors thereof, lubricants, mordants, matting agents, antistatic agents, plasticizers and other various kinds of additives which are useful for photographic light-sensitive materials. Typical examples of these additives are described in Research Disclosure, RD Nos. 17643 (December, 1978) and 18716 (November, 1979).

The silver halide emulsions which can be used in the present invention are those of silver bromide, silver chlorobromide and silver chloride which are substantially free from any silver iodide; and preferred silver halides are silver chlorobromide containing 20 to 98 mol% of silver bromide.

Particularly, to still more rapid processing, silver chlorobromide containing more than 80 mol% of silver chloride is preferably used.

The silver halide grains to be used in the present invention may comprise different inner and surface layer phases, or may have a multiphase constitution with epitaxial structure, or otherwise, may have a wholly uniform phase. Further, the present grains may comprise a combination of these structures.

The average grain size of the silver halide grains to be used in the present invention is preferably 0.1 µm to 2 µm, especially preferably 0.15 µm to 1 µm. (The grain size is the grain diameter in the case of spherical or nearly spherical grains or is the side length in the case of cubic grains, and the average grain size is represented on the basis of the mean value of the projected area of the grains.) The grain size distribution may be either narrow or broad. In particular, a so-called monodispersed silver halide emulsion is preferably used in the present invention, where the value of the standard deviation in the grain size distribution curve of the silver halide emulsion as divided by the average grain size thereof (or, that is, coefficient of variation) can fall within 20% or less, especially preferably 15% or less. In order to satisfy the desired gradation of the photographic light-sensitive materials, two or more monodispersed silver halide emulsions (where the monodispersed system preferably has the above-defined variation coefficient) having substantially the same color sensitivity but having different grain size distributions can be incorporated in the same layer or into plural different layers as laminated. Further, two or more kinds of polydispersed silver halide emulsions or a combination of a monodispersed emulsion and a polydispersed emulsion can be used in mixture or in laminate.

The shape of the silver halide grains to be used in the present invention may be a cubic, octahedral, dodecahedral, tetradecahedral or the like regular crystal, or may be a spherical or the like irregular crystal or, otherwise, the present grains may comprise composite forms of these crystal shapes. Cubic, tetradecahedral or the like regular crystal grains are preferably used. Further, the present grains may be tabular and, in particular, an emulsion where in 50% or more of the total projected area of the grains comprise tabular grains having an aspect ratio (length/thickness) of 5 or more, especially 8 or more, can be used in the present invention. An emulsion comprising a mixture of these various kinds of crystal forms can, of course, be used. These various kinds of emulsions may belong to either a surface latent image type where a latent image is formed essentially on the surface of the grains or an internal latent image type where a latent image is formed essentially in the inner part of the grains. The surface latent image type silver halide emulsion is preferably used in the present invention.

The photographic emulsions to be used in the present invention can be prepared by a variety of methods, for example, as described in P. Glafkides, Chimie et Physique Photographique (Paul Montel Co., 1967), G.F. Duffin, Photographic Emulsion Chemistry (Focal Press Co., 1966) and V.L. Zelikman et al., Making and Coating Photographic Emulsion (Focal Press Co., 1964). For instance, the present emulsions can be obtained by any of an acidic method, a neutral method, or an ammonia method; and for the reaction of a soluble silver salt and a soluble halide, a single jet method, a double jet method or a combination thereof can be utilized. A so-called reverse mixing method where the grains are formed in the presence of excess silver ions can also be utilized. Further, a so-called controlled double jet method which is one type of the double jet method can also be utilized, where the pAg value in the liquid phase to form the silver halide grains is kept constant. According to this method, silver halide emulsions having a regular crystalline form and a nearly uniform grain size can be obtained.

In addition, emulsions as prepared by a conversion method comprising a step for converting the already formed silver halide grains into those having a smaller solubility product during the procedure up to the completion of the formation of the silver halide grains, or emulsions as prepared by a method where the same halogen conversion is applied to the already formed grains after completion of the formation of the grains, can also be used.

For example a cadmium salt, a zinc salt, a lead salt, a thallium salt, an iridium salt or a complex thereof, a rhodium salt or a complex thereof and an iron salt or a complex thereof can exist for preventing the reciprocity law failure, e.g. increasing the sensitivity and controlling the gradation in the step for the formation of the silver halide grains or the physical ripening thereof.

The silver halide grains are generally subjected to physical ripening, demineralization or chemical ripening, after the formation thereof, and then coated on a support.

Known silver halide solvents (for example, ammonia, rhodankali or thioethers and thione compounds as described in U.S. Patent 3,271,157 and Japanese Patent Application (OPI) Nos. 12360/76, 82408/78, 144319/78, 100717/79 and 155828/79) can be used in precipitation, physical ripening and chemical ripening. The removal of soluble silver salts from the physically ripened emulsions can be carried out by noodle washing, flocculation precipitation or ultrafiltration.

The silver halide emulsions to be used in the present invention can be sensitized by a sulfur sensitization method where in sulfur-containing compound capable of reacting with an active gelatin or silver (for example, thiosulfates, thioureas, mercapto compounds and rhodanines) are used; a reductive sensitization method where in reducing substances (for example, stannous salts, amines, hydrazine derivatives, formamidine sulfinic acid, silane compounds) are used; or a noble metal sensitization method where in metal compounds (for example, gold complexes as well as complexes of the Periodic Table VIII group metals such as Pt, Ir, Pd, Rh, Fe) are used; and these sensitization methods can be utilized singly or in the form of a combination thereof.

Among these chemical sensitization methods, the single sulfur sensitization is more preferred.

Each of the blue-sensitive, green-sensitive and red-sensitive emulsions of the present invention are spectrally sensitized with methine dyes or the like other dyes so as to have the respective color sensitivity. Usable dyes include cyanine dyes, merocyanine dyes, complex cyanine dyes, complex merocyanine dyes, holopolar cyanine dyes, hemicyanine dyes, styryl dyes and hemioxonol dyes. Especially useful dyes are those belonging to cyanine dyes, merocyanine dyes and complex merocyanine dyes. Any and every basic heterocyclic nucleus which may generally be contained in cyanine dyes may be applied to these dyes. For instance, such nuclei include pyrroline, oxazoline, thiazoline, pyrrole, oxazole, thiazole, selenazole, imidazole, tetrazole and pyridine nuclei; alicyclic hydrocarbon ring-fused heterocyclic nuclei; and aromatic hydrocarbon ring-fused heterocyclic nuclei such as indolenine, benzindolenine, indole, benzoxazole, naphthoxazole, benzothiazole, naphthothiazole, benzoselenazole, benzimidazole and quinoline nuclei. These nuclei may be substituted on their carbon atoms.

Merocyanine dyes and complex merocyanine dyes may contain a ketomethylene structure-containing 5- or 6-membered heterocyclic nucleus, such as pyrazolin-5-one, thiohydantoin, 2-thiooxazolidine-2,4-dione, thiazolidine-2,4-dione, rhodanine or thiobarbituric acid nucleus.

These sensitizing dyes can be used singly or in the form of a mixture thereof, and the combination of the sensitizing dyes is often utilized for the purpose of supersensitization. Typical examples thereof are described in U.S. Patents 2,688,545, 2,977,229, 3,397,060, 3,522,052, 3,527,641, 3,617,293, 3,628,964, 3,666,480, 3,672,898, 3,679,428, 3,703,377, 3,769,301, 3,814,609, 3,837,862 and 4,026,707, British Patents 1,344,281 and 1,507,803, Japanese Patent Publication Nos. 4936/68 and 12375/78, and Japanese Patent Application (OPI) Nos. 110618/77 and 109925/77.

Dyes which themselves have no spectral sensitization activity or substances which do not substantially absorb visible rays but have a supersensitization activity can be incorporated into the emulsions together with the sensitizing dyes.

The present invention will be explained in greater detail by reference to the following examples. It should be understood that processing steps wherein the amount of benzyl alcohol exceeds 0.5 ml/l lie outside the scope of the claims.

### EXAMPLE 1

35 mℓ of ethyl acetate and 12 mℓ of Comparative Compound A (dielectric constant: 3.61) were added to 24.0 g of Yellow Coupler (Y-1) and dissolved, and the resulting solution was added to 160 mℓ of a 12% gelatin aqueous solution containing 12 mℓ of 10% sodium dodecylbenzenesulfonate, and emulsified and dispersed with a high speed stirrer to obtain an emulsified dispersion containing dispersed grains having a mean grain diameter of 0.46 µm. (The grain size was measured by the use of a grain size measuring apparatus with laser ray-scattering.) The total amount of the resulting dispersion was added to a silver chlorobromide emulsion comprising 80% of Br (Ag content: 70 g/kg), and the resulting emulsion was coated on a paper support laminated on both sides thereof with polyethylene, the coated Ag amount being 0.31 g/m², and a gelatin layer was provided over the thus coated layer to obtain Sample No. 1. Sodium 1-hydroxy-3,5-dichloro-s-triazine was used as the gelatin hardener.

Next, other emulsified dispersions as shown in the following Table 1 were prepared in the same manner as above, with the exception that the compound as shown below was used in place of Comparative Compound A and that the emulsification conditions were varied (by the variation of the rotation number of the stirring blades in emulsifier and the time for the emulsification) and, thus, Sample Nos. 2 through 10 were obtained in the same manner as the formation of Sample No. 1. The compounds used were as follows: Comparative Compound B (dielectric constant: 3.63)
Comparative Compound (S-7) (dielectric constant: 4.80)
Comparative Compound (S-9) (dielectric constant: 4.46)
Compound (S-16) (dielectric constant: 7.33)

Further, Sample Nos. 13 through 18 and Sample Nos. 21 through 26 were formed in the same manner as Sample Nos. 1 through 10 with the exception that a Magenta Coupler (M-1) and a Cyan Coupler (C-1) were used, respectively, in place of a Yellow Coupler (Y-1). In the case of the use of the magenta coupler, the amount of the coated coupler was 0.37 g/m², and the Ag-coated amount of the silver chlorobromide emulsion (Br content: 75 mol%) was 0.20 g/m²; and in the case of the use of the cyan coupler, the amount of the coated coupler was 0.33 g/m², and the Ag-coated amount of the silver chlorobromide emulsion (Br content: 70 mol%) was 0.28 g/m².

### Comparative Compound (S-7)

### Comparative Compound (S-9)

### Yellow Coupler (Y-1)

### Magenta Coupler (M-1)

### Cyan Coupler (C-1)

### Comparative Compound A (dielectric constant: 3.61)

### Comparative Compound B (dielectric constant: 3.63)

O=P(̵OC₁₈H₃₅)₃

These samples were subjected to gradation exposure for sensitometry and thereafter processed by the following Step (A) or (B), each using the following Color Developer (A) or (B), respectively. Steps (A) and (B) were the same with the differentiation of only the use of Color Developer (A) or (B) in each step.

The evaluation of the photographic properties was made on the two items of the maximum density (Dmax) and the minimum density (Dmin).

The results are given in Table 1.

| Processing Step | Temperature (°C) | Time (min) |
|---|---|---|
| Development | 38 | 2.0 |
| Bleach-Fixing | 33 | 1.5 |
| Rinsing | 28-35 | 3.0 |

### Composition of Developer:

### Color Developer (A):

| | |
|---|---|
| 3Na• Nitrilotriacetate | 2.0 g |
| Benzyl Alcohol | 15 mℓ |
| Diethylene Glycol | 10 mℓ |
| Na₂SO₃ | 2.0 g |
| KBr | 0.5 g |
| Hydroxylamine Sulfate | 3.0 g |
| 4-Amino-3-methyl-N-ethyl-N-[β-(methanesulfonamido)ethyl]-p-phenylenediamine Sulfate | 5.0 g |
| Na₂CO₃ (monohydrate) | 30.0 g |
| Water to make | 1,000 ml |
| | (pH 10.1) |

### Color Developer (B):

| | |
|---|---|
| 3Na•Nitrilotriacetate | 2.0 g |
| Na₂SO₃ | 2.0 g |
| KBr | 0.5 g |
| Hydroxylamine Sulfate | 3.0 g |
| 4-Amino-3-methyl-N-ethyl-N-[β-(methanesulfonamido)ethyl]-p-phenylenediamine Sulfate | 5.0 g |
| Na₂CO₃ (momohydrate) | 30.0 g |
| Water to make | 1,000 m² |
| | (pH 10.1) |

### Composition of Bleach-Fixing Solution:

| | |
|---|---|
| Ammonium Thiosulfate (54 wt%) | 150 mℓ |
| Na₂SO₃ | 15 g |
| NH₄[Fe(III) (EDTA)] | 55 g |
| EDTA•2Na | 4g |
| Water to make | 1,000 mℓ |
| | (pH 6.9) |

Table 1 proves that Sample No. 18 of the present invention had sufficient maximum density both in Step (A) and in Step (B) while the decrease in color density was especially noticeable in the comparative samples when processed in Step (B) with no benzyl alcohol.

### EXAMPLE 2

A multilayer color photographic paper of the present invention was formed, having the layers as shown in the following Table 2, the layers being provided on a paper support laminated on both sides thereof with polyethylene.

This light-sensitive material was designated as Sample (a).

The coating solutions were prepared as follows:

### Preparation of the First Layer-Coating Solution:

27.2 mℓ of ethyl acetate and 7.9 mℓ of Solvent (c) were added to 19.1 g of Yellow Coupler (a) and 4.4 g of Color Image Stabilizer (b) and dissolved. The resulting solution was added to 185 mℓ of a 10% gelatin aqueous solution containing 16 mℓ of 10% sodium dodecylbenzenesulfonate and emulsified in a homogenizer to obtain an emulsified dispersion having a mean grain diameter of 0.15 µm. (The grain size was measured by the use of a grain size measuring apparatus with laser ray-scattering.)

On the other hand, the following blue-sensitive sensitizing dye was added to a silver chlorobromide emulsion (silver bromide content: 80 mol%, silver content: 70 g/kg) in an amount of 7.0 x 10⁻⁴ mol per mol of the silver chlorobromide to obtain 90 g of a blue-sensitive emulsion.

The emulsified dispersion and the emulsion were blended and dissolved, and the gelatin concentration was regulared as shown in Table 2 to obtain a first layer-coating solution.

The other second layer- to seventh layer-coating solutions were prepared in the same manner as the first layer-coating solution.

Sodium 1-hydroxy-3,5-dichloro-s-triazine was used as the gelatin hardener in each layer.

The spectral sensitizer as used in each emulsion was as follows:

### Blue-Sensitive Emulsion Layer:

(7.0 x 10⁻⁴ mol per mol of silver halide was added)

### Green-Sensitive Emulsion Layer:

(4.0 x 10⁻⁴ mol per mol of silver halide was added) (7.0 x 10⁻⁵ mol per mol of silver halide was added)

### Red-Sensitive Emulsion Layer:

(1.0 x 10⁻⁴ mol per mol of silver halide was added)

The anti-irradiation dye as used in each layer was as follows:

### Green-Sensitive Emulsion Layer:

### Red-Sensitive Emulsion Layer:

The couplers and other compounds as used in the present example have the following structural formulae:
(a) Yellow Coupler (Y-35):
(b) Color Image Stabilizer:
(c) Solvent:
(d) Color Stain Preventing Agent:
(e) Magenta Coupler (M-23):
(f) Color Image Stabilizer:
(g) Solvent:
   Mixture (2/1 by weight) of and (dielectric constant : 7.33)
(h) Ultraviolet Absorbent:
   Mixture (1/5/3 by molar ratio) of the following: and
(i) Color Stain Preventing Agent:
(j) Solvent:
(k) Cyan Coupler:
(ℓ) Color Image Stabilizer:
   Mixture (1/3/3 by molar ratio) of the following: and
(m) Solvent: (S-16)

### Support:

Polyethylene laminated paper (containing white pigment of TiO2 and bluish dye of ultramarine in the polyethylene on the side supporting the first layer)

Next, the following Photographic Light-Sensitive Material Samples (b) through (d) were formed.

### Sample (b):

This was the same as Sample (a) with the exception that the mean grain sizes of the emulsified dispersions in each of the first, third and fifth layers were varied as shown in the following Table 3 by regulating the emulsification conditions of the dispersions.

### Sample (c):

This was the same as Sample (a) with the exception that the solvents in the first, third and fifth layers were replaced by the same volume of Comparative Compound A.

### Sample (d):

This was the same as Sample (c) with the exception that the mean grain sizes of the emulsified dispersions in each of the first, third and fifth layers were varied as shown in the following Table 3 by regulating the emulsification conditions of the dispersions.

These samples were subjected to gradation exposure for sensitometry through each of the blue, green and red filters with a sensitometer having a light source color temperature of 3,200°K. The exposure time was 0.5 s and the exposure amount was 250 CMS.

Afterwards, the thus exposed samples were processed by the following Step (A) or (B) with Color Developer (A) or (B), respectively, as shown below.

The photographic process comprised color development, bleach-fixing and rinsing; and the photographic characteristics of the samples were evaluated by varying the development 1 min, 2 min, and 3 min. Steps (A) and (B) were the same with the differentiation of only the use of Color Developer (A) or (B) in each step.

The evaluations of the photographic characteristics were made on four items of relative sensitivity, gradation, maximum density (Dmax) and minimum density (Dmin).

The relative sensitivity was represented by a relative value on the basis of the index value (100) of the sensitivity of each sample as processed by Step (A) wherein the color development time was 2 min . The sensitivity was designated by the relative value of the reciprocal of the exposure amount as required for obtaining the density comprising the minimum density plus 0.5.

The gradation was designated by the density difference between the sensitivity point and the point comprising the logarithm of the exposure amount (logE) plus 0.5.

The results are given in Table 3.

| Processing Step | Temperature (°C) | Time (min) |
|---|---|---|
| Development | 38 | 1.0-3.0 |
| Bleach-Fixing | 33 | 1.5 |
| Rinsing | 28-35 | 3.0 |

### Composition of Developer:

### Color Developer (A):

| | |
|---|---|
| 3Na•Nitrilotriacetate | 2.0 g |
| Benzyl Alcohol | 15 mℓ |
| Diethylene Glycol | 10 mℓ |
| Na₂SO₃ | 2.0 g |
| KBr | 0.5 g |
| Hydroxylamine Sulfate | 3.0 g |
| 4-Amino-3-methyl-N-ethyl-N-[β-(methanesulfonamido)ethyl]-p-phenylenediamine Sulfate | 5.0 g |
| Na₂CO₃ (monohydrate) | 30.0 g |
| Water to make | 1,000 mℓ |
| | (pH 10.1) |

### Color Developer (B):

| | |
|---|---|
| 3Na•Nitrilotriacetate | 2.0 g |
| Xa₂SO₃ | 2.0 g |
| KBr | 0.5 g |
| Hydroxylamine Sulfate | 3.0 g |
| 4-Amino-3-methyl-N-ethyl-N-[β-(methanesulfonamido) ethyl]-p-phenylenediamine Sulfate | 5.0 g |
| Na₂CO₃ (monohydrate) | 30.0 g |
| Water to make | 1,000 mℓ |
| | (pH 10.1) |

### Composition of Bleach-Fixing Solution:

| | |
|---|---|
| Ammonium Thiosulfate (54 wt%) | 150 mℓ |
| Na₂SO₃ | 15 g |
| NH₄[Fe(III)(EDTA)] | 55 g |
| EDTA•2Na | 4 g |
| Water to make | 1,000 mℓ |
| | (pH 6.9) |

Table 3 proves that the Photographic Light-Sensitive Material Sample (a) of the present invention is superior to the other Comparative Photographic Light-Sensitive Material Samples (b) through (d) in that the difference of the photographic properties(including relative sensitivity, gradation and maximum density) is small in Process (A) and Process (B) and thus the same result as in Process (A) can be attained even by Process (B) with no benzyl alcohol.

In addition, good photographic properties could be obtained by the development with a development time of 2 min in the present Sample (a).

### EXAMPLE 3

Samples (e), (f), (g) and (h) were prepared in the same manner as described for Samples (a), (b), (c) and (d), respectively, except that silver halide emulsions used for the first layer (blue-sensitive layer), the third layer (green-sensitive layer), and the fifth layer (red-sensitive layer) were a silver chlorobromide emulsion (silver bromide: 1 mol%, cubic shape, mean grain size: 1.0 µm), a silver chlorobromide emulsion (silver bromide: 1.5 mol%, cubic shape, mean grain size: 0.4 µm), and a silver chlorobromide emulsion (silver bromide: 1.5 mol%, cubic shape, mean grain size: 0.5 µm), respectively.

These samples were exposed as in Example 2, and then processed by the following Step (C) or (D) with Color Developer (C) or (D), respectively, as shown below to obtain color images.

Steps (C) and (D) were the same with the differentiation of only the use of Color Developer (C) or (D) in each step.

The evaluations of the photographic characteristics were made on two items of maximum density (Dmax) and minimum density (Dmin).

The results are given in Table 4 below.

| Processing Step | Temperature | Time |
|---|---|---|
| | (°C) | (sec) |
| Development | 35 | 45 |
| Bleach-Fixing | 30-35 | 45 |
| Rinsing* (1) | " | 20 |
| " (2) | | 20 |
| " (3) | " | 20 |
| " (4) | " | 30 |
| Drying | 70-80 | 60 |

| | | |
|---|---|---|
| *: Four stage countercurrent flow system is applied in rinsing stage. | | |

### Composition of Developer:

### Color Developer (C):

| | |
|---|---|
| Ethylenediamine-N,N,N',N'-tetramethylenephosphonic Acid | 1.5 g |
| 1,4-Diazabicyclo[2,2,2]octane | 6.0 g |
| Sodium Chloride | 1.4 g |
| Potassium Carbonate | 25 g |
| N-Ethyl-N-(β-methanesulfonamidoethyl)-3-methyl-4-aminoaniline Sulfate | 5.0 g |
| N,N-Diethylhydroxylamine | 4.2 g |
| Fluorescent Brightener (4,4'-diaminostilbene type) | 2.0 g |
| Benzyl Alcohol | 10.0 mℓ |
| Water to make | 1,000 mℓ |
| | (pH 10.10) |

### Color Developer (D):

This was the same as Color Developer (C) with the exception that benzyl alcohol is not contained.

### Composition of Bleach-Fixing Solution:

| | |
|---|---|
| Ammonium Thiosulfate (70 wt%) | 100 mℓ |
| Na₂SO₃ | 18 g |
| NH₄[Fe(III)(EDTA)] | 55 g |
| EDTA•2Na | 3 g |
| Ammonium Bromide | 40 g |
| Glacial Acetic Acid | 8 g |
| Water to make | 1,000 mℓ |
| | (pH 5.5) |

### Rinsing Solution:

Demineralized water (containing not more than 3 ppm of calcium and magnesium, respectively).

**TABLE 4**

| Sample | * Layer | Mean Grain Size of Emulsified Dispersion (µm) | Step (C)** | | Step (D)*** | | ΔDmax |
|---|---|---|---|---|---|---|---|
| | | | Dmin | Dmax | Dmin | Dmax | |
| (e) Invention | B | 0.11 | 0.10 | 2.21 | 0.10 | 2.18 | 0.03 |
| | G | 0.12 | 0.10 | 2.81 | 0.10 | 2.75 | 0.06 |
| | R | 0.12 | 0.11 | 2.89 | 0.11 | 2.85 | 0.04 |
| (f) Comparison | B | 0.32 | 0.10 | 2.20 | 0.10 | 2.01 | 0.19 |
| | G | 0.32 | 0.10 | 2.79 | 0.10 | 2.60 | 0.19 |
| | R | 0.31 | 0.12 | 2.87 | 0.11 | 2.70 | 0.17 |
| (g) Comparison | B | 0.12 | 0.10 | 2.10 | 0.10 | 1.80 | 0.30 |
| | G | 0.13 | 0.11 | 2.72 | 0.10 | 2.51 | 0.21 |
| | R | 0.14 | 0.11 | 2.84 | 0.11 | 2.62 | 0.22 |
| (h) Comparison | B | 0.32 | 0.10 | 2.09 | 0.10 | 1.73 | 0.36 |
| | G | 0.34 | 0.11 | 2.71 | 0.10 | 2.46 | 0.25 |
| | R | 0.32 | 0.12 | 2.82 | 0.10 | 2.53 | 0.29 |

| | | | | | | | |
|---|---|---|---|---|---|---|---|
| Note *: B: first layer in Samples (e) to (h) G: third layer in Samples (e) to (h) R: fifth layer in Samples (e) to (h) | | | | | | | |
| ** Comparison | | | | | | | |
| *** invention | | | | | | | |

Table 4 proves that the Photographic Light-Sensitive Material Sample (e) of the present invention is superior to the other Comparative Photographic Light-Sensitive Material Samples (f) through (h) in that the coloring property is high and the difference of the photographic properties of Step (C) and that of Step (D) is small.

Good photographic properties could be obtained by the development with a short development time and no benzyl alcohol in the present Sample (e).

## Claims

1. A method for the formation of colour images comprising image-wise exposing a silver halide colour photographic material having at least one silver halide emulsion layer on a reflective support, said emulsion layer containing a dispersion of oleophilic fine grains having a mean grain size of 0.05 to 0.25 µm which dispersion contains a pyrazolo[5,1-c]-[1,2,4]triazole or pyrazolo[1,5-b]-[1,2,4]triazole coupler capable of forming a magenta dye after having been coupled with an oxidation product of an aromatic primary amine developing agent, and at least one high boiling organic solvent having a dielectric constant of 5.0 or more (25°C, 10 kHz) and having the following formula (I) wherein W₁, W₂ and W₃ each represents a substituted or unsubstituted alkyl, cycloalkyl, alkenyl, aryl or heterocyclic group; and then subjecting the image-wise exposed photographic material to development with a colour developer which contains an aromatic primary amine developing agent and 0.5 ml/l or less of benzyl alcohol, for a period of time within 2 min and 30 s or less.

2. The method of claim 1, wherein W₁, W₂ and W₃ in the formula (I) each represents an unsubstituted alkyl, cycloalkyl, alkenyl, aryl, or heterocyclic group.

3. The method of claim 1, wherein W₁, W₂ and W₃ in the formula (I) each represents an alkyl group, a cycloalkyl group, an alkenyl group, an aryl group or a heterocyclic group as substituted by substituents(s) having one or more linking groups selected from the group consisting of -COO-, -CON〈, -R⁸N〈, and -0-, where R⁸ represents a divalent to hexavalent group derived from a phenyl group by removal of hydrogen atom(s) therefrom.

4. The method of claim 1, wherein W₁, W₂ or W₃ in the formula (I) represents a linear or branched alkyl group optionally substituted by one or more substituents selected from a halogen atom, a cycloalkyl group, an aryl group and an ester group.

5. The method of claim 1, wherein the high boiling organic solvents of the formula (I) have a viscosity of 20 mPa.s or more at 25°C.

6. The method of claim 1, wherein the colour developer contains no benzyl alcohol.

7. The method of claim 1, wherein the colour development time is 1 to 2 min.

8. The method of claim 1, wherein the oleophilic fine grains have a mean grain size of 0.05 µm to 0.20 µm.

9. The method of claim 1, wherein the colour developer is an alkaline aqueous solution mainly comprising the aromatic primary amine type colour developing agent.

10. The method of claim 1, wherein the processing temperature of the colour developer is 30 to 50°c.

11. The method of claim 1, wherein the processing temperature of the colour developer is 33 to 45°C.

12. The method of claim 4, wherein the ester group is a dibasic acid ester group, a lactate-derived group, a citrate-derived group, a malate-derived group, a tartrate-derived group and -CH₂-C(COOC₈H₁₇)(OH)-CH₂COOC₈H₁₇.

13. The method of claim 1, wherein the ratio by weight of the high boiling organic solvent to the coupler is from 0.05/1 to 20/1.

14. The method of claim 1, wherein the silver halide colour photographic material further contains an alkali metal halide or an organic fog inhibitor.

15. The method of claim 1, wherein the silver halide emulsion layer contains silver halide grains having a cubic or tetradecahedral crystal form.

16. The method of claim 1, wherein said silver halide emulsion layer contains a silver halide emulsion having a coefficient of variation of 20% or less.

17. The method of claim 16 wherein the coefficient of variation is 15% or less.

18. The method of claim 1, wherein the silver halide emulsion layer contains a silver chlorobromide from 20 to 98 mol% of silver bromide content, but having substantially no iodide.

19. The method of claim 1, wherein the silver halide emulsion layer contains a silver chloride or a silver chlorobromide having a silver chloride content of more than 80 mol%.

20. The method of claim 1, wherein the silver halide emulsion layer contains a silver halide emulsion which predominantly forms a latent image on the surface thereof upon exposure to light.

21. The method of claim 1, wherein the aromatic primary amine developing agent is 3-methyl-4-amino-N-ethyl- N-β-hydroxyethylaniline or 3-methyl-4-amino-N-ethyl-N-β-methanesulfonamidoethylaniline.

## Patentansprüche

1. Verfahren zur Herstellung von Farbbildern, das die folgenden Schritte aufweist: bildweises Belichten eines farbphotographischen Silberhalogenid-Materials mit mindestens einer Silberhalogenid-Emulsionsschicht auf einem reflektierenden Träger, wobei die Emulsionsschicht eine Dispersion oleophiler feiner Körner enthält, die eine mittlere Korngröße von 0,05 bis 0,25 µm aufweisen, wobei die Dispersion einen Pyrazolo[5,1-c]-[1,2,4]triazol- oder Pyrazolo[1,5-b]-[1,2,4]triazol-Kuppler enthält, der fähig ist, einen Magenta-Farbstoff zu bilden, nachdem er mit einem Oxidationsprodukt eines aromatischen primären Amin-Entwicklungsmittels gekuppelt wurde und mindestens ein hochsiedendes organisches Lösungsmittel mit einer dielektrischen Konstante von 5,0 oder mehr (25°C, 10 kHz) mit der folgenden Formel (I) wobei W₁, W₂ und W₃ jeweils eine substituierte oder unsubstituierte Alkyl-, Cycloalkyl-, Alkenyl-, Aryl- oder eine heterocyclische Gruppe bedeuten; und dann das Entwickeln des bildweisen belichteten photographischen Materials mit einem Farbentwickler, der ein aromatisches, primäres Aminentwicklungsmittel und 0,5 ml/l oder weniger Benzylalkohol enthält über eine Zeitspanne von 2 min und 30 s oder weniger.

2. Verfahren gemäß Anspruch 1, worin W₁, W₂ und W₃ in der Formel (I) jeweils eine unsubstituierte Alkyl-, Cycloalkyl-, Alkenyl-, Aryl- oder eine heterocyclische Gruppe bedeuten.

3. Verfahren gemäß Anspruch 1, worin W₁, W₂ und W₃ in der Formel (I) jeweils eine Alkylgruppe, eine Cycloalkylgruppe, eine Alkenylgruppe, eine Arylgruppe oder eine heterocyclische Gruppe bedeuten, substituiert mit einem oder mehreren Substituenten, die eine oder mehrere Verbindungsgruppen aufweisen, ausgewählt aus der Gruppe, bestehend aus -COO-, -CON〈, -R⁸N〈, und -O-, worin R⁸ eine divalente bis hexavalente Gruppe bedeutet, abgeleitet von einer Phenylgruppe durch Entfernung des/der Wasserstoffatoms(e).

4. Verfahren gemäß Anspruch 1, worin W₁, W₂ und W₃ in der Formel (I) eine lineare oder verzweigte Alkylgruppe bedeuten, gegebenenfalls substituiert durch ein oder mehrere Substituenten, ausgewählt aus einem Halogenatom, einer Cycloalkylgruppe, einer Arylgruppe und einer Estergruppe.

5. Verfahren gemäß Anspruch 1, worin die hochsiedenden organischen Lösungsmittel der Formel (I) eine Viskosität von 20 mPa·s oder mehr bei 25°C aufweisen.

6. Verfahren gemäß Anspruch 1, worin der Farbentwickler keinen Benzylalkohol enthält.

7. Verfahren gemäß Anspruch 1, worin die Farbentwicklungsdauer 1 bis 2 min beträgt.

8. Verfahren gemäß Anspruch 1, worin die oleophilen feinen Körner eine mittlere Korngröße von 0,05 µm bis 0,2 µm aufweisen.

9. Verfahren gemäß Anspruch 1, worin der Farbentwickler eine alkalische, wäßrige Lösung ist, die im wesentlichen das aromatische, primäre, aminartige Farbentwicklungsmittel enthält.

10. Verfahren gemäß Anspruch 1, worin die Verarbeitungstemperatur des Farbentwicklers 30 bis 50°C beträgt.

11. Verfahren gemäß Anspruch 1, worin die Verarbeitungstemperatur des Farbentwicklers 33 bis 45°C beträgt.

12. Verfahren gemäß Anspruch 4, worin die Estergruppe eine 2-basische Säureestergruppe ist, eine von Lactat abgeleitete Gruppe, eine von Citrat abgeleitete Gruppe, eine von Malat abgeleitete Gruppe, eine von Tartrat abgeleitete Gruppe und -CH₂-C(COOC₈H₁₇)(OH)-CH₂COOC₈H₁₇.

13. Verfahren gemäß Anspruch 1, worin das Gewichtsverhältnis des hochsiedenden organischen Lösungsmittels zum Kuppler zwischen 0,05 zu 1 bis 20 zu 1 liegt.

14. Verfahren gemäß Anspruch 1, worin das Silberhalogenidfarbphotographische Material weiterhin ein Alkali-Metallhalogenid oder einen organischen Schleierinhibitor enthält.

15. Verfahren gemäß Anspruch 1, worin die Silberhalogenid-Emulsionsschicht Silberhalogenidkörner enthält, die eine kubische oder tetradekahedrische Kristallform aufweisen.

16. Verfahren gemäß Anspruch 1, worin die Silberhalogenidemulsionsschicht eine Silberhalogenidemulsion mit einem Variationskoeffizienten von 20% oder weniger enthält.

17. Verfahren gemäß Anspruch 16, worin der Variationskoeffizient 15% oder weniger beträgt.

18. Verfahren gemäß Anspruch 1, worin die Silberhalogenid-Emulsionsschicht ein Silberchlorbromid mit 20 bis 98 Mol-% Silberbromidgehalt enthält, das aber im wesentlichen kein Iodid aufweist.

19. Verfahren gemäß Anspruch 1, worin die Silberhalogenid-Emulsionsschicht ein Silberchlorid oder ein Silberchlorbromid mit einem Silberchloridgehalt von mehr als 80 Mol-% aufweist.

20. Verfahren gemäß Anspruch 1, worin die Silberhalogenid-Emulsionschicht eine Silberhalogenid-Emulsion enthält, die vorrangig ein latentes Bild auf ihrer Oberfläche nach Belichtung bildet.

21. Verfahren gemäß Anspruch 1, worin das aromatische, primäre Aminentwicklungsmittel 3-Methyl-4-amino-N-ethyl-N-β-hydroxyethylanilin oder 3-Methyl-4-amino-N-ethyl-N-β-methansulfonamidoethylanilin ist.

## Revendications

1. Procédé pour la formation d'images couleur comprenant l'exposition selon une image d'un matériau photographique couleur à l'halogénure d'argent ayant au moins une couche d'émulsion d'halogénure d'argent sur un support réfléchissant, ladite couche d'émulsion contenant une dispersion de grains fins oléophiles ayant une taille moyenne de grain de 0,05 à 0,25 µm, laquelle dispersion contient un coupleur pyrazolo[5,1-c][1,2,4]triazole ou pyrazolo[1,5-b][1,2,4]-triazole capable de former un colorant magenta après avoir été couplé avec un produit d'oxydation d'un développateur de type amine aromatique primaire, et au moins un solvant organique à point d'ébullition élevé ayant une constante diélectrique de 5,0 ou plus (25°C, 10 kHz) et ayant la formule (I) suivante : dans laquelle W₁, W₂ et W₃ représentent chacun un groupe alkyle, cycloalkyle, alcényle, aryle ou hétérocyclique substitué ou non substitué ; puis la soumission du matériau photographique exposé selon une image à un développement avec un révélateur chromogène qui contient un développateur de type amine aromatique primaire et 0,5 ml/l d'alcool benzylique ou moins pendant une durée de 2 min et 30 s ou moins.

2. Procédé selon la revendication 1, dans lequel W₁, W₂ et W₃ dans la formule (I) représentent chacun un groupe alkyle, cycloalkyle, alcényle, aryle ou hétérocyclique non substitué.

3. Procédé selon la revendication 1, dans lequel W₁, W₂ et W₃ dans la formule (I) représentent chacun un groupe alkyle, un groupe cycloalkyle, un groupe alcényle, un groupe aryle ou un groupe hétérocyclique substitué par un ou plusieurs substituants ayant un ou plusieurs groupes de liaisons choisis dans le groupe constitué de -COO-, -CON〈, -R⁸N〈 et -O-, où R⁸ représente un groupe divalent à hexavalent dérivé d'un groupe phényle par élimination de l'un ou de plusieurs de ses atomes d'hydrogène.

4. Procédé selon la revendication 1, dans lequel W₁, W₂ ou W₃ dans la formule (I) représente un groupe alkyle linéaire ou ramifié éventuellement substitué par un ou plusieurs substituants choisis parmi un atome d'halogène, un groupe cycloalkyle, un groupe aryle et un groupe ester.

5. Procédé selon la revendication 1, dans lequel les solvants organiques à point d'ébullition élevé de formule (I) ont une viscosité de 20 mPa.s ou plus à 25°C.

6. Procédé selon la revendication 1, dans lequel le révélateur chromogène ne contient pas d'alcool benzylique.

7. Procédé selon la revendication 1, dans lequel le temps de développement couleur est de 1 à 2 min.

8. Procédé selon la revendication 1, dans lequel les grains fins oléophiles ont une taille moyenne de grain comprise entre 0,05 µm et 0,20 µm.

9. Procédé selon la revendication 1, dans lequel le révélateur chromogène est une solution aqueuse alcaline comprenant principalement le développateur chromogène de type amine aromatique primaire.

10. Procédé selon la revendication 1, dans lequel la température de traitement du révélateur chromogène est de 30 à 50°C.

11. Procédé selon la revendication 1, dans lequel la température de traitement du révélateur chromogène est de 33 à 45°C.

12. Procédé selon la revendication 4, dans lequel le groupe ester est un groupe ester d'acide dibasique, un groupe dérivé de lactate, un groupe dérivé de citrate, un groupe dérivé de malate, un groupe dérivé de tartrate et -CH₂-C(COOC₈H₁₇)(OH)CH₂COOC₈H₁₇.

13. Procédé selon la revendication 1, dans lequel le rapport en poids du solvant organique à point d'ébullition élevé au coupleur est de 0,05/1 à 20/1.

14. Procédé selon la revendication 1, dans lequel le matériau photographique couleur à l'halogénure d'argent contient de plus un halogénure de métal alcalin ou un inhibiteur de voile organique.

15. Procédé selon la revendication 1, dans lequel la couche d'émulsion d'halogénure d'argent contient des grains d'halogénure d'argent ayant une forme cristalline cubique ou tétradécaédrique.

16. Procédé selon la revendication 1, dans lequel ladite couche d'émulsion d'halogénure d'argent contient une émulsion d'halogénure d'argent ayant un coefficient de variation de 20 % ou moins.

17. Procédé selon la revendication 16, dans lequel le coefficient de variation est de 15 % ou moins.

18. Procédé selon la revendication 1, dans lequel la couche d'émulsion d'halogénure d'argent contient un chlorobromure d'argent ayant une teneur en bromure d'argent de 20 à 98 mol% mais ne contenant pratiquement pas d'iodure.

19. Procédé selon la revendication 1, dans lequel la couche d'émulsion d'halogénure d'argent contient un chlorure d'argent ou un chlorobromure d'argent ayant une teneur en chlorure d'argent de plus de 80 mol%.

20. Procédé selon la revendication 1, dans lequel la couche d'émulsion d'halogénure d'argent contient une émulsion d'halogénure d'argent qui forme principalement une image latente à sa surface lors d'une exposition à la lumière.

21. Procédé selon la revendication 1, dans lequel le développateur de type amine aromatique primaire est la 3-méthyl-4-amino-N-éthyl-N-β-hydroxyéthylaniline ou la 3-méthyl-4-amino-N-éthyl-N-β-méthanesulfonamidoéthylaniline.
